

Nov. 12, 1929.

O. J. NELSON

1,735,440

ART OF RECLAIMING LUBRICATING OILS

Filed Jan. 8, 1923



Inventor

OLIVER J. NELSON,  
by John H. Bruninga.  
His Attorney.

## UNITED STATES PATENT OFFICE

OLIVER J. NELSON, OF ST. LOUIS, MISSOURI, ASSIGNOR TO BRYTE-NELSON REFINING COMPANY, OF ST. LOUIS, MISSOURI, A CORPORATION OF MISSOURI

## ART OF RECLAIMING LUBRICATING OILS

Application filed January 8, 1923. Serial No. 611,308.

This invention relates to the reclaiming of lubricating oils, and more particularly those oils having a mineral base and which have been used in crank cases of gas engines.

(50%) of lighter hydrocarbons, thereby reducing the viscosity to such an extent that it may only be one-twentieth (1/20) of that of the original oil. These lighter hydrocarbons are found in practice to be about mid-way between gasoline and kerosene. 55

5 The lubricating oil used in crank cases has a mineral base but the composition of this lubricant base varies. Thus where it is obtained from a paraffin base petroleum, it is the residue remaining after distillation of the 10 lighter and heavier hydrocarbons, while if the petroleum has an asphaltic or mixed base, it is the distillate following the volatilization of the naphthas and kerosene. In the compounding of lubricating oils, the viscosity and 15 body are often raised by the addition of cylinder stock, animal fats and oils and vegetable oils. Sometimes even soaps and mere adulterants are added. Accordingly in a given crank case the mixture may be complex 20 not only from the standpoint of the original mineral oils due to the constant addition of different grades and makes, but the mixture may also contain compounds other than mineral oil.

Solid matter, such as carbon, metal grindings and particles, earthly matter and sand also enter the crank case. Furthermore moisture will frequently enter with the fuel, 60 as when a cylinder is missing or when starting. Accordingly under the churning action in the crank case, complex emulsions and colloids are formed, more especially where animal fats and alkalis are present, as is frequently the case where the viscosity and body 65 are raised by the addition of fats and soaps.

The result, therefore, is that the mixture in a crank case is a very complex one. Moreover where the oil from a number of crank 70 cases is dumped into a common vat, the resultant mixture is even more complex.

25 The oil in a crank case is subject to unusual treatment while in use. Upon reciprocation the oil is splashed on the cylinder walls and is caused to spread over the same in a film. As this film is exposed to high temperatures, the 30 oil may be cracked and this cracked product is then washed down into the crank case, not only by the wiping action of the piston and the washing action of the oil, but also by the action of unvolatilized fuel and condensed 35 moisture which enter the crank case past the pistons. The oil in the crank case is furthermore subjected to considerable heat due to conduction as well as escape of gases from the combustion chamber into the crank case.

40 Since the oil is churned and exposed to air under the influence of heat, the result is an oxidation and polymerization so that asphaltic and resinous compounds are formed. 75

It has been attempted to reclaim the oil from such a mixture, but previous processes have not on the whole been successful in view of the fact that the complex nature and the required treatment have not been fully appreciated and understood. Such a complex mixture cannot be treated like the original petroleum, whether of a paraffin, asphaltic 80 or mixed base, because the mixture contains various foreign substances and is in a different condition than is the case with petroleums. A mere filtering or acid treatment is not sufficient; nor can the ordinary 85 processes of distillation be utilized. The reclaiming of such a used lubricating oil, containing as it does solid matter, moisture and lighter hydrocarbons partially emulsified and polymerized, requires knowledge of the 90 composition and nature of the mixture and the treatment necessary in order to meet the conditions.

45 With the employment of the lower grade fuel now used and the tendency of running an engine cold, frequent priming and missing of cylinders, a good deal of the volatile hydrocarbons are washed down into the crank case, diluting the oil therein to such an extent that 50 the body may contain as much as fifty percent

95 It has been found by experiment that the lubricating property of the mineral base is not damaged by use, even under the strenuous conditions encountered in a crank case, but that the value of the mineral base has been rather enhanced, because what has remained behind has been due to the survival 100

of the fittest part. The complex mixture, however, requires the most careful treatment.

From an economic stand point the reclamation of such lubricating oil is exceedingly important for the reason that the oil under 5 adverse conditions in the crank case loses its lubricating value very readily so that it must be changed and discarded with great frequency. Accordingly there are millions 10 of barrels of such lubricating oil discarded every year, which is not only a loss to the industry, but its disposal is moreover troublesome and costly since it cannot be run into sewers on account of the danger of explosion 15 and fire.

One of the objects of this invention, therefore, is to provide a process of treatment of such a lubricating oil whereby the mineral base will not only be reclaimed and regenerated, but conserved in such a manner as to 20 obtain as result a lubricant which is even of a higher grade than the original lubricants.

Further objects will appear from the 25 tail description taken in connection with the accompanying drawing, in which the figure is an elevation partly in section. The description and drawing illustrate an embodiment of this invention. It will be noted, 30 however, that in the drawing parts have not only been illustrated diagrammatically but not necessarily at the proper elevations, as this drawing is simply for illustration and is not intended to show the actual arrangement and location of the elements of the 35 plant.

In accordance with this invention, the used lubricating oil is subjected generally to the following treatments, namely: a defecating or 40 clarifying treatment, a distillation treatment and a filtering treatment. Furthermore the body is also allowed to cool between the distillation and filtering treatments.

The character of the clarifying or defecating treatment depends upon the character 45 and condition of the oil and upon the foreign bodies which it contains as well as upon the nature of the incorporation of these bodies within the mineral oil base. If the oil body contains only solid particles and mechanically entrained water, a simple centrifuging 50 may be sufficient, especially if it is preceded by a heat treatment, especially by an agitating heat treatment with steam.

Usually, however, the oil body contains the solid matter and the water in a difficult 55 separable form and more especially in the form of complex emulsions or colloids, so that mere centrifuging even if preceded by a heat treatment is not sufficient. In such a case the oil body is subjected to an acid treatment while agitated with air, followed by an alkali treatment while agitated with air and then steam, followed by settling, the upper 60 portion being then again agitated with live

steam and the body so treated is then centrifuged.

In the distilling treatment, the body of oil is gradually heated over an extended period, the first stage being a rather gentle heat, while the body is gently agitated with air followed by more violent agitation with air. Live steam is then gradually blown into the body along with the air and thereafter the air is gradually cut down while the steam is increased 70 until nothing but steam enters the body. The steam is now superheated, preferably by the heat of the body of oil itself, until the temperature rises preferably above the vaporizing point of the mineral base so 75 that some of this mineral base begins to pass over with the steam. The heating is now interrupted and the oil body is allowed to settle slowly in order to cool to a temperature considerably below the volatilization point of 80 the mineral base. The oil body is then drawn from the still and cooled to a point where it will not ignite.

The cooled oil body is now filtered, preferably through fuller's earth and this filtering 85 is under pressure and at a temperature sufficient to cause the oil to flow through the filter.

In order to more clearly describe the invention, an example of a practical embodiment 90 of this invention and of a plant illustrating a practical embodiment for carrying out the process will be given; it is to be understood, however, that the construction and arrangement may be varied without departing from the spirit of this invention. Furthermore it will be understood that the drawing is illustrative only and in somewhat 95 diagrammatical form and that it does not necessarily show the parts in their true positions. Furthermore pipes and valves are 100 shown in conventional form and will not be referred to in detail.

Referring now to the accompanying drawing, 1 designates a vat of a suitable construction to permit treatment of the oil with sulphuric acid and alkali. It is provided with a perforated pipe 2 which may have an air connection 3 and a steam connection 4, whereby either air or steam or both may be blown 110 through the connections therein. Suitable supply lines 5 and 6 may be provided for a mineral acid, such as sulphuric acid, and an alkali, such as caustic soda. The vat discharges into a settling tank 7 and from this tank the upper portion is taken by a pipe 8 to a treating tank 9 provided with a heating coil 10, receiving steam from the boiler 11. This tank also contains a perforated pipe 12 also connected to receive steam. The vat 9 115 discharges into a steam operated centrifuge 13 which in turn has a spout 130 discharging into a storage tank 14.

From the storage tank 14 a pump 15 delivers the body to a still 16, which is preferably 120

arranged on a brick foundation of a furnace having a combustion chamber 17 heated by a fuel burner 18, which may be either of the oil or gas type. The still is provided with a 5 heating coil 19 connected with the steam pipe 20 and with the exhaust 21. The bottom of the still further has arranged therein a perforated pipe 22, the perforations of which extend along the lower side so as to direct 10 jets of air or steam on the bottom of the still, and this pipe has suitable valve connections with the steam pipe 20 and the exhaust 21 and a suitable air connection with an air pipe 23. The top of the still has a large 15 vapor pipe 24 which is horizontally arranged and of large capacity and connects with an upper branch 25 and a lower branch 26 connected by legs 27. The branches 25 and 26 are practically horizontal, draining slightly to 20 the right or away from the still. The outlet 24 as well as the top and side of the furnace are preferably jacketed with an insulating material to retain the heat and thus avoid condensation. The bottom of the still has 25 an outlet 28.

From the still the pipes 25 and 26 lead to a condenser 29 which may be of the water cooled type and from this condenser the condensates are led to storage tanks 30.

30 The body of the oil is taken from the still by a pump 31 through cooling coils 32 into a storage tank 33. From the storage tank a pump 34 takes the oil to the pressure filters 35. These filters contain a suitable filtering 35 material 36 such as fuller's earth, and each is provided with a steam heating coil 37 and with an air pressure connection 38.

Assuming that used lubricating oil from crank cases is the body to be treated, and 40 that this oil contains impurities and is in the condition as previously described, the general operation of a practical embodiment of a process embodying this invention is as follows:

45 The usual lubricating oil is placed in the tank or vat 1 and sulphuric acid of about 66° Bé. is added in the proportion of about five to seven pounds to a barrel of the oil. This is then agitated with air for about two hours.

50 The function of this treatment is to partially dissolve any metal particles, break up the emulsions and colloids, and cause precipitation of the solid matter due to the breaking up of the emulsion. The acid treatment further 55 acts to break up the polymerized products and more especially those of an asphaltic and a resinous nature. The body is now neutralized with a concentrated caustic soda solution of 30° to 33° Bé. and is agitated first

60 with air and then with live steam for about two hours at a temperature of about 105° F. This treatment not only neutralizes the sulphuric acid and other acids which may be present, but the steam in condensing also 65 dries the alkali and all dissolved impurities

which are now contained in the water entrained with the oil.

The body so treated is now allowed to settle for about twenty-four hours in the vat 7, which causes settling of a great part of the 70 solid matter and a part of the water, especially that entrained mechanically as well as some resulting from the breaking up of the emulsions and colloids.

The heavier matter will settle to the bottom 75 while the less dense part containing the oil floats on top. The upper portion is now removed to the vat 9 where it is agitated and heated with live steam to about 150° F. This thoroughly mixes the different components 80 of the oil. It not only renders the body more suitable for the subsequent centrifuging but further serves to assist in the breaking up of the emulsion, especially those that may be formed by the addition of the caustic soda 85 and by the treatment with live steam.

The body is now subjected to the action of the centrifuge 13 which further serves to remove the heavier impurities and water and serves to additionally effect breaking up of 90 the emulsions. It is, however, found that even all of the impurities and water will not be removed but that about five percent may remain. The centrifuge discharges into the 95 vat 14 which is simply a storage vat.

The body is now pumped into the still 16 which is filled 85% full. It is now first subjected to a slow heat while the body is agitated with air for a period of about twenty 100 minutes, until the temperature is raised slightly above the boiling point of water, that is, to about 212 to 215 degrees F. During this procedure the body is gradually heated and some of the volatile matter in the form of dissolved gases may pass off and some moisture is also freed. Some of the emulsion may also be partially broken up and carried off with the air. This air performs the function of not only keeping the mass in motion so as to cause uniform heating, but water settling 110 to the bottom will be blown up through the oil body and carried off with the air in the form of vapor. This air will also prevent foaming and bumping.

The still is now heated so that its temperature will be gradually elevated over a period of about three hours from 215° F. to 700° F. During this gradual heating the procedure is as follows and the oil passes through various 120 stages:

While the temperature is rising from 215° to 265° F., the body is blown with air at a pressure at about 10 to 15 pounds per square inch. This serves not only to blow out moisture but also carry out all entrained gases. It also causes oxidation of any oxidizable products which may be present and which, when formed into gas, are carried off with the air. The direction of the air blasts on the bottom of the still furthermore prevents 130

burning of the oil where it is in contact with the hot walls next to the fire.

When the temperature reaches 265° F., live steam is passed in with the air so that both steam and air will issue from the pipe 22. While the temperature is rising from 265° to 320° F., the air is gradually cut down while the live steam is increased until at the end of this particular stage and when the temperature reaches 320° F., live steam alone will issue from the pipe and will be directed against the bottom of the still, thereby not only securing thorough mixing of the oil but also preventing scorching.

During this stage the lighter hydrocarbons, such as gasoline and naptha are volatilized and pass out with the steam, and since these lighter hydrocarbons pass out during the latter part of the stage, the presence of the wet steam will prevent ignition and explosion of these lighter hydrocarbons. Of course, the presence of the steam will reduce the boiling point of the lighter hydrocarbons so that they will be volatilized at a lower temperature than if the steam were not present. This is important in the reclamation of lubricating oil, since it is necessary that the heat be as low as possible in order that as little decomposition may take place as possible, in order to obtain the highest viscosity and the least amount of cracking. The steam in stirring the oil further prevents local overheating and the vapors as soon as formed are carried off by the steam so that they do not fall back into the hot oil. Furthermore the arrangement of the pipe 24 and the jacketing of the same are such that the gases will pass out freely without any liability of condensing and falling back into the hot oil. In this way cracking is entirely avoided, which is desirable since cracking not only reduces the lubricating oil content but also causes the formation of objectionable asphaltic and resinous products.

When the temperature reaches 320° F. the live steam connection to the pipe 22 is cut off and the steam is passed first through the coil 19 and then into the pipe 22. This causes the steam before it issues from the pipe 22 to pass through the body of the oil so that it will become superheated. During this stage the temperature rises to 700° F. and at the end of the stage the pressure rises to 125 pounds per square inch. Accordingly the steam has a superheat of 350° F. During this stage the heavy napthas and kerosene and animal fats pass off and are carried over with the steam and there is also a complete breaking up of any asphaltic and resinous matter which may be present. The distillation is continued until the mineral base begins to pass over, which is determined by the distillate having a gravity of from 30° to 32° Bé, and by the fact that half of the vapors passing over is steam.

At the end of this stage all of the hydrocarbons and fats as well as water, which are more volatile than the mineral base, will have been distilled from the body, while any other impurities present will be completely broken up. The still contents are now allowed to settle until the temperature drops to 500° F., a little steam in a superheated condition, being passed through the body in order to keep up the temperature and keep the mass in agitation so that this cooling down is extended over a period of about one hour. This not only prevents cracking but insures that all the hydrocarbons and fats of lower volatilization than the mineral base will have passed off, that other impurities will be completely broken up and separated from the mineral base and that the whole is mixed and worked to form a uniform mass. The oil is now drawn from the still through cooling coils 32, which reduces the temperature to about 100° F. and thence to a storage tank 33.

The oil is pumped from the storage tank 33 to the filters 35 containing fuller's earth, through which the oil is passed under pressure of about seventy-five pounds per square inch, while maintained at a temperature of from 100 to 110° F., this filtering serving to filter out coloring matter and any residue which may remain, more particularly any asphaltic or resinous matter which may have been separated from the oil body.

The oil issuing from the filters is a high grade lubricating oil, having a high viscosity, high flash point and high fire test together with better adhesive and cohesive properties than even paraffin mineral bases. As an example, the treatment as heretofore described of a complex lubricating oil collected in St. Louis from automobile garages, resulted in a purified product whose viscosity was found to be 280 seconds (Saybolt), and had a flash point of 500° F., a fire test of 525° F. and a density of 29½° to 30° Bé.

While certain theories of operation have been advanced, it is to be understood that the purpose has been one of explanation and not of limitation, since it is not essential that the operation be dependent upon any theory, for the description of the above process is of an actual practical and existing embodiment. It is, therefore, to be understood that this invention is not to be limited to any theory advanced. It is further obvious that various changes may be made in details without departing from the spirit of this invention; it is, therefore, to be understood that this invention is not to be limited to any details described or shown.

Having thus described the invention, what is claimed is:

1. In the art of reclaiming used mineral lubricating oil containing solid matter, moisture, fats and lighter hydrocarbons, and partially emulsified and polymerized, the

process comprising, defecating the oil to clear the same of the solid matter and entrained water, heating the defecated oil at a temperature and for a period sufficient while agitated with air so as to remove the remaining moisture, heating the same at a temperature and for a period sufficient while agitated with steam to remove the fats and lighter hydrocarbons, and filtering the residue.

10 2. In the art of reclaiming used mineral lubricating oil containing solid matter, moisture and lighter hydrocarbons, and partially emulsified and polymerized, the process comprising, defecating the oil to clear the same of the solid matter and entrained water, gradually heating the defecated oil to the vaporizing point of the mineral lubricant base for a period sufficient to volatilize the remaining moisture and lighter hydrocarbons, blowing the oil body while being so heated, first with air and then with steam, and filtering the residue.

15 3. In the art of reclaiming used mineral lubricating oil containing solid matter, moisture and lighter hydrocarbons, and partially emulsified and polymerized, the process comprising, defecating the oil to clear the same of the solid matter and entrained water, gradually heating the defecated oil to the vaporizing point of the mineral lubricant base for a period sufficient to volatilize the remaining moisture and lighter hydrocarbons, blowing the oil body while being so heated, first with air, then with a mixture of air and steam and then with steam alone, and filtering the residue.

20 4. In the art of reclaiming used mineral lubricating oil containing solid matter, moisture and lighter hydrocarbons, and partially emulsified and polymerized, the process comprising, defecating the oil to clear the same of the solid matter and entrained water, gradually heating the defecated oil to the vaporizing point of the mineral lubricant base for a period sufficient to volatilize the remaining moisture and lighter hydrocarbons, blowing the oil body while being so heated, first with air, then with a mixture of air and live steam, and then with superheated steam alone, and filtering the residue.

25 5. In the art of reclaiming used mineral lubricating oil containing solid matter, moisture and lighter hydrocarbons, and partially emulsified and polymerized, the process comprising, defecating the oil to clear the same of the solid matter and entrained water, gradually heating the defecated oil to the vaporizing point of the mineral lubricant base for a period sufficient to volatilize the remaining moisture and lighter hydrocarbons, blowing the oil body while being so heated, first with air, then with a mixture of air and steam and then with steam alone, permitting the body to cool while agitated with steam, and filtering the residue.

6. In the art of reclaiming used mineral lubricating oil containing solid matter, moisture and lighter hydrocarbons, and partially emulsified and polymerized, the process comprising, defecating the oil to clear the same of the solid matter and entrained water, gradually heating the defecated oil to the vaporizing point of the mineral lubricant base for a period sufficient to volatilize the remaining moisture and lighter hydrocarbons, blowing the oil body while being so heated, first with air, then with a mixture of air and live steam and then with superheated steam, permitting the body to cool while agitated with superheated steam, and filtering the residue.

7. In the art of reclaiming used mineral lubricating oil containing solid matter, moisture and lighter hydrocarbons, and partially emulsified and polymerized, the process comprising, treating the oil body with a mineral acid, treating the same with an alkali, gradually heating the oil body so treated to the vaporizing point of the mineral lubricant base, blowing the oil body while so heated, first with air, then with a mixture of air and steam and then with steam alone, and filtering the residue.

In testimony whereof I affix my signature

this 27th day of December, 1922.

OLIVER J. NELSON.

100

105

110

115

120

125

130